

## 1

3,489,551

 ABRASION RESISTANT FERROUS ALLOY  
CONTAINING CHROMIUM

Stewart G. Fletcher and Walter T. Haswell, Jr., Latrobe, Pa., assignors to Latrobe Steel Company, a corporation of Pennsylvania  
No Drawing. Continuation-in-part of application Ser. No. 429,621, Feb. 1, 1965. This application July 30, 1968, Ser. No. 748,632

Int. Cl. C22c 39/26

U.S. Cl. 75—126

4 Claims

10

## ABSTRACT OF THE DISCLOSURE

An abrasion resistant readily workable alloy is provided comprising carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium about 1.1% to about 5%, sulfur up to about 0.25%, and the balance iron with residual impurities in ordinary amounts, said titanium being combined with carbon in a weight ratio of 4:1 and the vanadium with carbon in a weight ratio of 4.2 (V—1):1.

This application is a continuation-in-part of our pending application Ser. No. 429,621 filed Feb. 1, 1965 now abandoned.

This invention relates to ferrous alloys and abrasion resistant articles thereof and particularly to a low cost abrasion resistant alloy which is readily workable and castable. The search for steels having high abrasion resistance and low cost, together with satisfactory workability, has been a long and continuing one. Examples of uses for such steels are brick mold liners, tile dies, said blast equipment, shot blast equipment and various forms of dies. Alloys generally available at a favorable cost are undesirably short-lived and less than satisfactory for abrasion-resisting purposes.

We have discovered an alloy having improved forge-

15

20

25

30

35

40

45

50

55

60

65

70

## 2

|            |       |     |
|------------|-------|-----|
| Molybdenum | ----- | 1.1 |
| Titanium   | ----- | 2   |
| Vanadium   | ----- | 2   |

Balance substantially iron with residual impurities in ordinary amounts, said titanium being combined with carbon in a weight ratio of 4:1 and said vanadium with carbon in a weight ratio of 4.2 (V—1):1.

The composition of our alloy may, however, extend over a relatively wide range and still retain its desirable properties of workability and abrasion-resistance. It may include alloying elements such as nickel, cobalt, tungsten and vanadium within certain limited amounts and proportions without detrimentally affecting the abrasion-resistance. Such wider range of composition may fall within the following limits:

|            |       |                         |
|------------|-------|-------------------------|
| Carbon     | ----- | About 1 to about 4.25%. |
| Silicon    | ----- | About 1.5% maximum.     |
| Manganese  | ----- | About 1.5% maximum.     |
| Chromium   | ----- | About 10% to about 15%. |
| Molybdenum | ----- | Less than 2%.           |
| Titanium   | ----- | About 0.5 to about 5%.  |
| Tungsten   | ----- | Less than 3%.           |
| Nickel     | ----- | Less than 3%.           |
| Cobalt     | ----- | Less than 5%.           |
| Vanadium   | ----- | About 1.1 to about 5%.  |
| Sulfur     | ----- | Up to 0.25%.            |

Balance substantially iron with residual impurities in ordinary amounts, said titanium being combined with carbon in a weight ratio of 4:1 and the vanadium with carbon in a weight ratio of 4.2 (V—1):1.

The expression "less than" followed by a percentage figure in this application, in the context of this application means that the particular element may be entirely absent or it may be present in an amount not to exceed the percentage concentration given. The presence of these elements is optional up to the amount specified in the ranges of composition given above.

In order to illustrate the improved properties of our new alloy, several heats were made within the range of composition herein specified and compared with steels previously used for making brick liners and the like. The compositions appear in Table I.

TABLE I

| Alloy               | C    | Cr    | W     | Mo   | Ti    | V    | Si   | Mn  | Ni    | Co    |
|---------------------|------|-------|-------|------|-------|------|------|-----|-------|-------|
| Invention WR71----- | 2.76 | 12.38 | ----- | 1.07 | 2.21  | 1.90 | 0.35 | .48 | ----- | ----- |
| Prior art-----      | 2.4  | 12.75 | ----- | 1.1  | ----- | 4    | 0.40 | .40 | ----- | ----- |

ability, workability and abrasion resistance over any alloys previously available to the metallurgical industry. Our invention provides an abrasion-resistant alloy in which carbon within certain limits, is added in excess of that previously available to the metallurgical industry. Our invention provides an abrasion-resistant alloy in which carbon within certain limits, is added in excess of that necessary to give a desired hardening ability to the alloy together with vanadium and titanium in certain proportions and within certain limits such that the excess carbon

Abrasion tests were made, comparing these several alloys with the results which appear in Table II.

Table II

|                 |                  |
|-----------------|------------------|
| 55 Alloy:       | Percent abrasion |
| WR71 -----      | 2.58             |
| Prior art ----- | 3.76             |

Careful comparison of the foregoing results shows the superiority of our alloy over the alloys now used for abrasion resistant purposes. Moreover, we have found that the compositions with titanium present are far more workable than like compositions in which vanadium has been completely substituted for titanium, so that titanium must appear as an essential ingredient at least in the minimum amount specified herein in order to attain the improved workability along with improved abrasion resistance which characterizes our invention.

While we have described and disclosed certain preferred embodiments of this invention, it will be understood that this invention may be otherwise embodied within the scope of the following claims.

|           | Percent |
|-----------|---------|
| Carbon    | 2.9     |
| Silicon   | 0.4     |
| Manganese | 0.4     |
| Chromium  | 12.5    |

$$\frac{V-1}{4.3} + \frac{Ti}{4}$$

Considering only the essential elements of our alloy, the preferred analysis for most abrasion-resisting applications is:

We claim:

1. An abrasion-resistant readily workable alloy capable of being worked and cast to ultimate shape comprising carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium about 1.1% to about 5%, sulfur up to about 0.25%, and the balance iron with residual impurities in ordinary amounts, said titanium and vanadium being combined with carbon in excess of that necessary to give a desired hardenability such that titanium is combined with carbon in a weight ratio of 4:1 and the vanadium with carbon in a weight ratio of 4.2 (V-1):1.

2. An abrasion-resistant readily workable alloy capable of being worked and cast to ultimate shape comprising carbon about 2.9%, silicon about 0.4%, manganese about 0.4%, chromium about 12.5%, molybdenum about 1.1%, titanium about 2%, vanadium 2%, sulfur up to about 0.25% and the balance iron with residual impurities in ordinary amounts, said titanium being combined with carbon in a weight ratio of 4:1 and the vanadium with carbon in a weight ratio of 4.2 (V-1):1.

3. An article made from a ferrous base metal comprising carbon about 1% to about 4.25%, silicon about 1.5% maximum, manganese about 1.5% maximum, chromium about 10% to about 15%, molybdenum less than about 2%, titanium about 0.5% to about 5%, tungsten less than about 3%, nickel less than about 3%, cobalt less than about 5%, vanadium about 1.1% to about 5%, sulfur up to about 0.25% and the balance iron with residual impurities in ordinary amounts, said titanium and vanadium being combined with carbon in excess of that necessary to give a desired hardenability in proportions such that said titanium is combined with carbon in a

weight ratio of 4:1 to form titanium carbide and the vanadium with carbon in a weight ratio of 4.2 (V-1):1 to form vanadium carbide, said alloy being characterized by workability, castability, abrasion resistance and high impact resistance.

5. An article of manufacture made from a ferrous base metal alloy capable of being worked and cast to ultimate shape comprising carbon about 2.9%, silicon about 0.4%, manganese about 0.4%, chromium about 12.5%, molybdenum less than about 2%, titanium about 0.5% to about 5%, tungsten less than about 3%, nickel less than about 3%, cobalt less than about 5%, vanadium about 1.1% to about 5%, sulfur up to about 0.25% and the balance iron with residual impurities in ordinary amounts, said titanium being combined with carbon in a weight ratio of 4:1, and the vanadium with carbon in a weight ratio of 4.2(V-1):1, said alloy characterized by workability, castability, abrasion resistance and high resistance to impact.

#### References Cited

#### UNITED STATES PATENTS

|           |         |         |       |           |
|-----------|---------|---------|-------|-----------|
| 1,599,425 | 9/1926  | McGuire | ----- | 75—126    |
| 2,147,121 | 2/1939  | Emmons  | ----- | 75—126    |
| 2,575,218 | 11/1951 | Giles   | ----- | 75—126    |
| 3,231,709 | 1/1966  | Foley   | ----- | 75—126 XR |
| 3,295,401 | 1/1967  | Rackoff | ----- | 75—126 XR |

#### OTHER REFERENCES

30. Tool Steels, 3rd ed., 1962, published by American Society for Metals, Metal Park, Ohio, pp. 699—704 and 718.

HYLAND BIZOT, Primary Examiner

U.S. Cl. X.R.

35 75—128

UNITED STATES PATENT OFFICE  
CERTIFICATE OF CORRECTION

Patent No. 3,489,551

January 13, 1970

Stewart G. Fletcher, et al.

It is certified that error appears in the above identified patent and that said Letters Patent are hereby corrected as shown below:

Column 1, line 38, "said" should read -- sand --; line 51, "availiable" should read -- available --; lines 54 to 56, cancel "previously available to the metallurgical industry. Our invention provides an abrasion-resistant alloy in which carbon within certain limits, is added in excess of that"; same column 1, lines 61 and 62, the equation should appear as shown below:

$$\frac{V-1}{4.2} + \frac{Ti}{4}$$

Column 2, line 7, "ration" should read -- ratio --.

Signed and sealed this 3rd day of November 1970.

(SEAL)

Attest:

EDWARD M. FLETCHER, JR.  
Attesting Officer

WILLIAM E. SCHUYLER, JR.  
Commissioner of Patents